

## UNITED STATES PATENT OFFICE

2,107,157

## EXPLOSIVE

Harold A. Lewis, Wilmington, Del., and Fred R. Wilson, Bloomfield, N. J., assignors to E. I. du Pont de Nemours & Company, Wilmington, Del., a corporation of Delaware

No Drawing. Application January 22, 1936.  
Serial No. 60,260

8 Claims. (Cl. 52—14)

This invention relates to a new and improved detonating explosive and more particularly to one adapted for use in coal mining where the production of coal in the form of large lumps is 5 desirable.

The blasting impulse which is imparted by the explosive to its environment is, in part, a function of the reaction rates of two closely related consecutive chemical reactions, namely: (1) the rate 10 of initiation of the explosive decomposition; and (2) the rate at which the explosive decomposition takes place after initiation. Based on the wide 15 differences in the reaction rates of various explosives, it is customary to classify them into (a) deflagrating explosives, in which the two rates mentioned above are relatively slow; and (b) detonating explosives, in which the two rates are generally extremely rapid.

The first of the two factors mentioned above 20 may be expressed in slightly different terms as the rate of propagation, or the rate at which the initiating impulse travels down a column of explosive. In the case of deflagrating explosives, the initiating impulse is a flame which travels down 25 a column of black powder, for example, at a rate of about 300 m./sec. For detonating explosives on the other hand, the initiating impulse is a shock such as a "detonation wave", which proceeds down a column of dynamite, for example, 30 at a velocity generally in excess of 1700 m./sec.

The rate of propagation of an explosion wave is 35 readily measured by fairly accurate methods which generally consist in measuring the time required for an explosion wave to pass from one point to another along a column of the explosive being tested, for example in the case of detonating explosives, by means of the well known Mette-gang Recorder or the Dautriche method.

The second factor in the blasting impulse, 40 namely, the rate at which the chemical decomposition takes place at a given point after the initiating impulse has reached that point and started the decomposition, is a true reaction rate and as such, is extremely difficult to determine 45 with accuracy. Some indication of the magnitude of this rate may be obtained by observing the pressure changes in a closed system and determining the so-called "rate of pressure development". Since this is a rapidly changing differential function, it is the common practice to determine the so-called "time of pressure development", or the time required for the explosive to 50 develop the maximum hot gas pressure, when suitably initiated.

The methods of measuring either the rate or

the time of maximum hot pressure development have not been standardized, and in the case of detonating explosives in particular, no reliable procedure is known whereby reproducible results may be obtained. Indeed, the data obtained by 5 the known methods are of such doubtful value as to be lacking in significance. For these reasons, the performance of the explosive in actual blasting is a more reliable indication of the 10 rate of pressure development than the results of comparative tests in a Bichel bomb, for example.

One of the most accurate of these field tests 15 is a statistical study of the amount and size of the lumps produced in the shooting of coal with the powder under evaluation. With typical deflagrating explosives, such as black powder for example, large amounts of lump coal will be produced, since the characteristically low velocity of the propagation and low rate of pressure development will produce a heaving rather than a shattering 20 effect on the material blasted down. With detonating explosives on the other hand, a greater proportion of pulverized material or "fines" 25 will be produced depending on the magnitude of the two rates mentioned above.

From the foregoing, it will be seen that deflagrating explosives such as black powder are 30 more satisfactory in coal shooting, from the point of view of execution, than the detonating explosives heretofore available, due to the greater 35 economic value of lump coal. Black powder has a characteristic disadvantage, however, of producing a flame of considerable length and duration, which makes this explosive out of the question for safety reasons in mines where inflammable gases are present.

For the reasons given above, coal mining operations frequently require a detonating explosive which may be safely used in fiery mines. For 40 such purposes the most approxed explosives are the so-called "permissible explosives" which are designated as such by the U. S. Bureau of Mines after passing certain prescribed and official tests.

The great majority of the so-called "permissibles" contain ammonium nitrate as the principal 45 ingredient. These ammonium nitrate "permissibles" generally comprise, for example, 50 to 80% ammonium nitrate, 10 to 15% nitroglycerine as a sensitizing ingredient, up to 10 and as high as 50 20% of carbonaceous combustible materials, and frequently additions of safety ingredients or cooling salts such as sodium nitrate, ammonium chloride, sodium chloride, ammonium oxalate and the like in varying percentages. Thus, for ex- 55

ample, in the case of sodium nitrate, the most commonly used safety ingredient, the percentage varies from about 3 to 10%.

Typical examples of "ammonia permissibles" according to the prior art are shown in Table I.

Table I

|    | A                                               | B     | C     | D     |       |
|----|-------------------------------------------------|-------|-------|-------|-------|
| 10 | Nitroglycerine.....                             | 10.0  | 11.0  | 11.0  | 14.0  |
|    | Ammonium nitrate.....                           | 75.0  | 78.5  | 75.0  | 65.5  |
|    | Safety ingredients.....                         | 5.5   | 3.0   | 4.0   | 3.0   |
|    | Carbonaceous combustibles.....                  | 9.2   | 7.2   | 9.7   | 17.2  |
|    | Antacid.....                                    | 0.3   | 0.3   | 0.3   | 0.3   |
| 15 |                                                 | 100.0 | 100.0 | 100.0 | 100.0 |
|    | Velocity, m./sec. ....                          | 2750  | 2200  | 1900  | 1850  |
|    | Density.....                                    | 1.0   | 1.0   | 0.8   | 0.65  |
| 20 | Nitroglycerine—grams per 100 cc. explosive..... | 10.0  | 11.0  | 8.8   | 9.1   |

From the safety standpoint, such permissible detonating explosives have given great satisfaction and they have been excellently adapted for use with many types of coal from the viewpoint of execution. In cases, however, where the coal is soft and offers little resistance, and where a high percentage of lump coal is desired, such explosives are too violent in their action to give the desired results. This violence of action, as above explained, is due in part to the velocity of propagation, but by far the more important factor is believed to be the rate of pressure development. Since, however, the rate of pressure development can only be inferred indirectly from the performance of the explosive in actual use in the field, the exact explanation of the failure of prior "permissibles" to give the desired results under these circumstances is not definitely known, but the explanation given above appears to be correct.

The object of the present invention is an improved detonating explosive adapted for use in coal mining and producing a relatively large percentage of lump coal. A further object is such an explosive characterized by high strength, but having at the same time a low rate of pressure development. A still further object is a detonating explosive having a very low velocity and a very low rate of pressure development. Additional objects will be disclosed as the invention is herein-after more fully described.

We have found that the foregoing objects are accomplished by introducing into the explosive composition ammonium nitrate in an amount at least equal to 65% and preferably 75 to 80%, said ammonium nitrate being so controlled as to grain size and so sensitized with nitroglycerine or other nitric esters as to make certain a velocity less than 1700 meters per second and a low rate of pressure development. The ammonium nitrate used is of such a degree of coarseness that substantially the greater part thereof (i. e. over 90%) is held on a 35-mesh screen, and preferably we find it desirable to use even coarser grains, such for example that substantially the greater proportion thereof (i. e. over 80%) is held on a 24-mesh screen. The sensitizer used, nitroglycerine or other explosive nitric esters, is used in an amount not exceeding 7.5 grams per 100 cc. of explosive, and preferably between 4.5 and 6.5 grams per 100 cc. of explosive.

As illustrative of the preferred ranges within which the various ingredients of our explosive may be used, reference is made to Table II.

Table II

| Ingredients                                     | A        | B        | C        | 5  |
|-------------------------------------------------|----------|----------|----------|----|
| Nitroglycerine.....                             | 4.5-6.5% | 6-8%     | 8-10%    |    |
| Ammonium nitrate.....                           | 75-85%   | 75-85%   | 65-75%   |    |
| Safety ingredients.....                         | 0-10%    | 0-10%    | 0-10%    |    |
| Carbonaceous combustibles.....                  | 4-10%    | 7-15%    | 10-20%   |    |
| Antacid.....                                    | 0.1-1.0% | 0.1-1.0% | 0.1-1.0% | 10 |
| Properties                                      |          |          |          |    |
| Density.....                                    | 1.0      | 0.8      | 0.65     |    |
| Nitroglycerine—grams per 100 cc. explosive..... | 4.5-6.5  | 4.8-6.4  | 5.2-6.5  | 15 |

In the foregoing table the ammonium nitrate employed is of a degree of coarseness such that substantially the greater part thereof (e. g., over 80%) passes a 10-mesh screen but is held on a 24-mesh screen.

In explosive compositions of the type shown in Table II there is a minimum amount of sensitizer which is necessary for detonation; this is usually 3.0 to 4.0 grams of sensitizer per 100 cc. of explosive. In practice, it is necessary to use an amount slightly above the minimum in order to obtain a practical explosive composition. On the other hand, if an amount of sensitizer is used that is too far above the necessary minimum, then the reactions are set up with such violence that the rate of pressure development is increased and thus adversely affected for the purposes of our invention. The compositions shown in Table II therefore all contain an amount of sensitizer less than 7.5 grams per 100 cc. and within the preferred range of 4.5 to 6.5 grams per 100 cc.

The safety ingredients preferably comprise sodium nitrate, but any other of the well known cooling salts may be used if desired. The carbonaceous combustibles may consist of oat hulls, corn meal, bran, ground coal, wood pulp, expanded cereal products, cottonseed hulls, rice hulls, ivory nut meal, starch, flour and the like, or any mixtures thereof. Preferably, however, we use those combustibles which give compositions of a high degree of sensitiveness, particularly in those compositions of low density. As an example of this type of combustible, we may mention flaked cereal products such as flaked corn, wheat, rye, starch, hominy grits and the like. The antacid may consist of calcium carbonate, magnesium carbonate, magnesium oxide and the like.

As specific examples of a "permissible" type explosive in accordance with our invention, we may cite the compositions illustrated in Table III.

Table III

| Ingredients                                     | A     | B     | C     | 60 |
|-------------------------------------------------|-------|-------|-------|----|
| Nitroglycerine.....                             | 5.0   | 7.0   | 9.0   |    |
| Ammonium nitrate.....                           | 84.0  | 80.0  | 71.0  |    |
| Sodium nitrate.....                             | 3.0   | 3.0   | 3.0   |    |
| Absorbent combustible.....                      | 7.5   | 9.5   | 16.5  | 65 |
| Chalk.....                                      | 0.5   | 0.5   | 0.5   |    |
|                                                 | 100.0 | 100.0 | 100.0 |    |
| Properties                                      |       |       |       |    |
| Velocity, m./sec.....                           | 1500  | 1520  | 1450  |    |
| Strength.....                                   | 58%   | 60%   | 51%   | 70 |
| Density.....                                    | 1.0   | 0.8   | 0.65  |    |
| Nitroglycerine—grams per 100 cc. explosive..... | 5.0   | 5.6   | 5.9   |    |

A typical screen analysis of the ammonium nitrate employed in the examples given in Table III is indicated in Table IV.

Table IV

|                      | Percent |
|----------------------|---------|
| Held on 10 mesh      | 1       |
| Held on 10-14 mesh   | 4       |
| 5 Held on 14-20 mesh | 49      |
| Held on 20-24 mesh   | 34      |
| Held on 24-28 mesh   | 8       |
| Held on 28-35 mesh   | 3       |
| Held on 35-65 mesh   | 1       |
| Held on 65-100 mesh  | 0       |
| Passing 100 mesh     | 0       |
| 10                   | 100.0   |

From the foregoing table it is apparent that 99% of the ammonium nitrate employed passed a 10-mesh screen and 88% thereof was held on a 15 24-mesh screen.

We are aware that "relatively coarse ammonium nitrate" has been used heretofore in explosive compositions. Thus Woodbury in U. S. 1,113,275 and 1,124,679 disclosed that the substitution of "relatively large particles" of ammonium nitrate for the random sizes employed before that time caused a significant lowering of the velocity of detonation. Ward in U. S. 1,743,172 disclosed that relatively coarse ammonium nitrate could be successfully detonated at full strength with as little as 4 to 7% nitroglycerine.

In particle size, the "relatively coarse" ammonium nitrate heretofore employed was such that at least 80% was held on a 60-mesh screen, and not more than 20% passed therethrough. Our invention, however, contemplates the use of much coarser ammonium nitrate, for example such that at least 80% is held on a 24-mesh screen.

At first glance, this may appear to be an inconsequential difference from the ammonium nitrate heretofore employed, for example by Woodbury and Ward. This increase in the particle size, however, produces the surprising result that the powders according to our invention have a much lower rate of pressure development, and therefore produce an appreciably higher percentage of lump coal. Heretofore no one appears to have recognized that the rate of pressure development of ammonia dynamites may be lowered by employing ammonium nitrate of very large particle sizes as above described. By actual tests, however, we have found this to be the case. This is clearly indicated in Table V.

Table V

|    | Explosive used             | Percent coal held on 2-inch mesh |
|----|----------------------------|----------------------------------|
| 55 | Composition A of Table I   | 32                               |
|    | Composition B of Table I   | 36                               |
|    | Composition A of Table III | 44                               |

Table V gives the results of a statistical study 60 of the percentage of "fines" produced by various "permissibles" when used to "pull" coal in the same mine under comparable blasting conditions. In this table the results obtained by the use of the composition A of Table III according to our invention are compared to those obtained with the prior art compositions A and B of Table I. It will be noted that whereas there was an increase of 4% of 2-inch lump coal obtained by the use of composition B of Table I having a velocity of 2200 meters as compared with composition A of Table I having a velocity of 2750 meters, there was an increase of 2-inch lump of from 36 to 44% when employing composition A of Table III 70 in accordance with our invention. This increase

of from 36 to 44% represents an actual increase of 22% in the lump coal produced.

As mentioned above, the velocities of compositions A, B and C in Table III are somewhat lower than the corresponding properties of the common prior art "permissibles". By far the more important change, however, resulting from the selection of grain sizes is an unexpected and very appreciable reduction in the rate of pressure development of the explosive, as indicated by actual tests 10 in the field, for example, as shown in Table V. An explosive such as those described in Table III will possess to an unexpected degree the properties necessary for producing lump coal and will have high strength, between 50% and 60% 15 straight dynamite, due to its high content of explosive material, namely, nitroglycerine and ammonium nitrate. The strength, however, will develop slowly because of the presence of ammonium nitrate in the form of very coarse grains. 20 The low nitroglycerine content will be insufficient to cause the rapid development of pressure from the coarse grains of ammonium nitrate, but will be ample to develop the maximum strength of the explosive when the latter is shot in cartridges 25 of sufficiently large diameter.

An explosive such as the foregoing is not consistently capable of detonation at its full explosive strength when shot in the smaller diameters usual in prior art coal blasting. It has been the 30 custom, for example, to consider cartridges of 1 1/4" diameter as a standard. Our explosive, however, cannot effectively be used in diameters appreciably lower than 1 1/4" since the danger of misfires is too great. Consequently, the utilization 35 of explosives according to our invention in diameters not less than 1 1/2" is a prerequisite, and preferably the cartridge should have a diameter of 1 3/4" or more.

It will be apparent to any one skilled in the 40 art that a notable advance has been made possible by our new explosive. The superior qualities of black powder in the breaking down of coal in the form of large lumps has long been recognized. To the best of our knowledge, however, the present invention is the first to recognize that detonating explosives of the dynamite type, containing 45 very large particles of ammonium nitrate, are capable of producing similar favorable results. Thus, by the use of our explosives, it is possible 50 to produce a significantly higher percentage of lump coal in the presence of fire-damp than has ever been achieved before with a permissible ammonium nitrate dynamite.

In the foregoing detailed description of our 55 invention, it is apparent that many changes and modifications may be introduced without departing from the spirit and scope thereof. For example, the term "nitroglycerine" as employed in this specification and the appended claims is used 60 in the sense in which it is employed in the art. i. e. it includes not only nitroglycerine as such, but the various explosive nitric esters commonly used in place of, or in mixtures with, nitroglycerine, for example ethyleneglycol dinitrate, tetra-nitrodiglycerine, nitrated sugars, nitrostarch, nitrochlorhydrins, pentaerythritol tetrinitrate and various mixtures of these and similar substances. In addition, aromatic nitrocompounds such as the dinitrotoluenes, the nitroxylenes, and the like, 65 and similar explosive materials may be added if desired. Furthermore, the liquid nitric esters may be slightly gelatinized if desired by the addition of small percentages of nitrocotton or other gelatinizing agents. Other variations will be ap-

parent to anyone skilled in the art. We, therefore, intend to be limited only in accordance with the following patent claims:

We claim:

- 5 1. An ammonium nitrate explosive charge adapted for use in coal mining, and having a low velocity and a low rate of pressure development, said explosive comprising more than 65% ammonium nitrate of a degree of fineness such that 10 substantially the greater part thereof will be held on a 24-mesh screen and substantially all thereof will be held on a 35-mesh screen, said explosive being cartridge in a diameter not less than 1½", whereby a substantially complete utilization of 15 the explosive strength of the ammonium nitrate is assured.
2. An ammonium nitrate explosive charge adapted for use in coal mining, and having a low velocity and a low rate of pressure development, 20 said explosive comprising at least 65% ammonium nitrate of a degree of fineness such that substantially all thereof will be held on a 35-mesh screen, and a sensitizing agent comprising not more than 7.5 grams explosive nitric ester per 100 cc. of explosive, said explosive being cartridge in a diameter not less than 1½", whereby a substantially 25 complete utilization of the explosive strength of the ammonium nitrate is assured.
3. An ammonium nitrate explosive charge 30 adapted for use in coal mining, and having a low velocity and a low rate of pressure development, said explosive comprising not more than 7.5 grams of nitroglycerine per 100 cc. of explosive, and at least 75% ammonium nitrate of a degree of fineness such that substantially all thereof will be held on a 35-mesh screen, said explosive being cartridge in a diameter not less than 1½", whereby a substantially 35 complete utilization of the explosive strength of the ammonium nitrate is assured.
4. An ammonium nitrate explosive charge 40 adapted for use in coal mining, and having a low

velocity and a low rate of pressure development, said explosive comprising 4.5 to 6.5 grams of nitroglycerine per 100 cc. of explosive and at least 75% ammonium nitrate of a degree of fineness such that substantially all thereof will be held on a 35-mesh screen, said explosive being packaged in a diameter not less than 1½" inches. 5

5. An ammonium nitrate explosive charge adapted for use in coal mining, and having a low rate of pressure development, said explosive comprising 10 4.5 to 6.5 grams of nitroglycerine per 100 cc. of explosive and from 75 to 85% ammonium nitrate of a degree of fineness such that substantially all thereof will be held on a 35-mesh screen, said explosive being packaged in a diameter not 15 less than 1½" and having a velocity lower than 1700 m./sec. 15

6. A high strength ammonium nitrate permissible-type explosive charge adapted for use in coal mining, and having a low rate of pressure development, comprising approximately 4.5 to 6.5 grams nitroglycerine per 100 cc. of explosive, 75 to 85% ammonium nitrate of a degree of fineness such that substantially the greater part thereof will be held on a 24-mesh screen and substantially all thereof will be held on a 35-mesh screen, 20 1 to 5% of sodium nitrate, 5.0 to 15% of a carbonaceous combustible which favors sensitiveness at low percentages of nitroglycerine, and 0.5% chalk, said explosive having a velocity lower than 25 1700 m./sec. and being cartridge in a diameter not less than 1½", whereby a substantially complete utilization of the explosive strength of the ammonium nitrate is assured. 30

7. The composition of claim 6, in which said carbonaceous combustible comprises a flaked cereal product. 35

8. The composition of claim 6, in which said carbonaceous combustible comprises a flaked corn product. 40

HAROLD A. LEWIS.  
FRED R. WILSON.